

## UNITED STATES PATENT OFFICE

2,383,511

COMPOSITE ALUMINUM-ALLOY SHEETS AND  
METHOD OF MAKING SAME

Richard S. Reynolds, Richmond, Va.

Application November 1, 1941, Serial No. 417,578

3 Claims. (Cl. 29—189)

The present invention has for its object to provide an aluminum-alloy sheet composed of layers of aluminum alloys of different characteristics and which are mutually resistant to bonding. As an example, certain aluminum alloys have marked resistance to fatigue and have relatively high yield strength, and yet do not possess substantial resistance to abrasion in handling. Other aluminum alloys lack the stated or other qualities and, at the same time, are highly resistant to abrasion. In order to combine in one structure the advantage of both alloys, it has been proposed to roll together assembled slabs of the alloys in order to produce a composite sheet, but this was established as impractical because of poor adherence.

I have discovered a method of overcoming the problem which has heretofore prevented the commercial production of such composite aluminum alloy sheets.

In the drawing I have diagrammatically shown a composite aluminum alloy sheet in which 1 represents a greatly enlarged alloy sheet, as, for example, of aluminum, copper, manganese and magnesium, and 2 indicates the commercially pure aluminum bond, 3 representing an alloy sheet, as, for example, aluminum silicon, magnesium and chromium.

As a specific example, for a basic alloy slab I may employ aluminum alloyed with copper, manganese and magnesium, such as in the approximate percentages of 4.2% copper, 0.6% manganese, and 1.5% magnesium. This alloy has a specific gravity of 2.76 and weight in pounds per cubic inch of 0.100. It is therefore light, and it has initial relatively high yield strength. When annealed, it has a hardness of 42 Brinell which is very substantially increased by heat treatment and quenching and by hot rolling. One primary characteristic of the alloy is its resistance to fatigue, which remains substantially constant, the factor not being substantially changed by heat treatment.

Continuing the specific example, for the associated alloy slab or slabs, I may employ aluminum alloyed with silicon, magnesium and chromium such as in the approximate percentages 0.7% silicon, 1.25% magnesium and 0.25% chromium. Such alloy material has a weight in pounds per cubic inch of 0.097 and a specific gravity of 2.69, with a hardness exceeding 40 Brinell in annealed state.

Between the basic and each associated slab, I interpose a layer of aluminum, pure or of standard commercial purity. Commercial pig alu-

minum contains small percentages of iron, silicon and copper, the latter two materials being in lesser degree and the total of these common alloys being upwards of 1%. Thus "commercially pure" aluminum may be employed for my bonding material.

Particularly, a scalped ingot of the so-called basic alloy, which may be of any desired thickness, such as 5", may have applied to the opposite faces thereof thinner plates or sheets such as plates of 0.250" composed of the associated alloy specified above. Intermediate the ingot and each of the associated plates, I interpose a sheet of commercially pure aluminum which may be .020" thick, that thickness being sufficient to insure exceedingly thin but uniform bonding layers in the final composite sheet.

The composite body, generally heated as in standard ingot rolling practice, is then rolled down to the thickness desired for the specific purpose as, for example, one of the customary sheet thicknesses extensively used in the aircraft industry.

By following this method, I have found that the layers are permanently bonded into an integral structure. In the specific example, the aluminum-alloy sheet thus produced embodies in one structure the advantageous qualities of both the base and the associated alloy structures, the surface exposed alloy associated with the basic alloy being resistant to abrasion and possessing other inherent characteristics, so that the composite body has marked advantages over a sheet made of the composite alloys, according to usual practice.

It will be understood that the specific example is used to illustrate the invention, and the invention is capable of wide application to the association of aluminum-alloy bodies which resist mutual bonding.

Having described my invention, what I claim and desire to secure by Letters Patent, is as follows:

1. A rolled composite metallic sheet comprising a plurality of hard aluminum-alloy layers exceeding 40 Brinell in hardness, the layers being characterized by resistance to mutual bonding under pressure, and intermediate each two layers a foil of commercially pure aluminum bonding the assembly into a permanent integral sheet structure, the aluminum bonding containing less than 1% silicon.
2. A composite metallic sheet comprising a plurality of hard aluminum-alloy layers exceeding 40 Brinell in hardness, and intermediate each

Aug. 28, 1945.

C. ROSENTHAL

2,383,512

## KNOCKDOWN COLLAPSIBLE CLOSET

Filed May 27, 1944

Fig. 1.



Fig. 2.



Fig. 3.



**INVENTOR**  
*Charles Rosenthal*

BY *Clark & Ott*  
ATTORNEYS

